

## UNITED STATES PATENT OFFICE

2,575,008

## METHOD OF CREPING NYLON

Abraham L. Dargin, New York, N. Y.

No Drawing. Application March 16, 1949,  
Serial No. 81,845

14 Claims. (Cl. 28—76)

1

This invention relates to the formation of a nylon crepe fabric.

An object of the invention is to provide a creped fabric without embossing or similar process and which, in its finished state, consists solely of nylon or any other similar synthetic yarn.

A further object is to provide a yarn of the character hereafter described which may be woven into fabrics along with other yarns to produce novel effects in the cloth.

I use a yarn which comprises nylon or similar synthetic yarn combined with raw silk in one thread. It may be thrown with half right twist and half left twist or with a one way twist. The number of turns given the yarn is determined substantially by the size of the thread desired. For example, the combination of a 40 denier filament yarn with one end of 20 to 22 denier raw silk would be given about 60 to 65 turns per inch. The silk would constitute about 25% to 50% of the yarn by weight.

This yarn is then used in the manufacture of fabrics either for warp, or filling, or both, depending upon the construction of the cloth desired.

The woven or knitted fabric is boiled off in the usual manner. This boiling off process causes the silk to shrink or contract. In shrinking or contracting, the silk contracts or crinkles the nylon or similar synthetic yarn with which it has been thrown imparting a creped or crinkled effect to the fabric. The nylon or similar synthetic yarn is then set in the aforementioned contracted position by the application of heat. The degree of heat applied depends on the type and construction of the fabric but for the reasons set forth below it is desirable that in all cases this degree of heat exceed the boiling point of water.

I have found that the boiling off process supplies sufficient heat to the nylon or other similar synthetic yarn to set it without the necessity of the setting procedure described above. However, the setting by the boil off process sets the nylon or similar synthetic yarn only to the extent of the degree of heat of boiling water, viz., 212° F. I prefer, therefore, after the boil off to set the nylon or similar synthetic yarn at a temperature in excess of the boiling point of water to avoid any possible damage in the laundering process of the finished garment.

The nylon or similar synthetic yarn having been set, it will retain its creped position and is no longer dependent upon the silk for this purpose.

Accordingly, the silk is dissolved by immersing the fabric in a hot caustic solution, the strength

2

of which depends upon the construction of the cloth itself. The fabric is then treated with an acid bath which neutralizes any of the caustic solution which may remain on the fabric. This caustic solution and acid bath may, if desired, be employed before the setting by the application of heat described above because as shown above, the boiling off process supplies a sufficient setting to the nylon or other similar synthetic yarn to allow for the removal of the silk after such setting.

The silk having been completely dissolved and removed from the fabric, the result is a fabric which is 100% nylon or similar synthetic yarn with a permanently set creped effect.

Fabrics, when made and finished as set forth above have all of the advantages of nylon or similar synthetic fabrics as heretofore made with the added advantage that the creped structure forms air pockets and therefore prevents the clinging of the garment to the body of the wearer.

A spun nylon may be used instead of a continuous filament with the same results.

It will be appreciated that many uses may be made of a fabric constructed in accordance with the aforesaid invention but the essential feature of the invention is the contracting and setting of the nylon or similar synthetic yarn so that it imparts a creped effect to the fabric.

Thrown silk may be used in the place and stead of raw silk.

It is of course possible to form the composite threads of nylon material and silk and treat them to contract the silk on the nylon thread to produce the creped effect, then treat the thus creped composite thread to remove the silk, and then form a fabric of the creped nylon threads, if desired.

40 I claim:

1. A method of making a fabric wholly of nylon which comprises forming a fabric with yarn consisting of nylon combined with silk, shrinking the silk to give a creped position to the nylon, setting the nylon in this creped position by the application of heat, and dissolving the silk to remove it from the fabric.

2. A method of making a nylon fabric which comprises forming a fabric with yarn consisting of nylon combined with silk, shrinking the silk to give a creped position to the nylon, and dissolving the silk to remove it from the fabric.

3. A method of making a fabric wholly of nylon yarn which comprises forming a fabric comprising nylon yarn combined with silk, shrinking the

silk to give the nylon a crinkled effect, and dissolving the silk to remove it from the fabric.

4. A method of making a creped fabric wholly of nylon which comprises forming a fabric with a yarn comprising nylon combined with silk in one thread, boiling off the fabric and shrinking the silk which in turn gives a crinkled position to the nylon, setting the nylon in this crinkled position by the application of heat and dissolving the silk and removing it from the fabric by immersing the fabric in a hot caustic solution and then in a neutralizing acid bath.

5. A method of making a fabric wholly of nylon yarn which comprises forming a fabric comprising such nylon yarn combined with silk in one thread, boiling off the fabric and shrinking the silk which in turn gives a creped position to the nylon yarn, setting the nylon yarn in this creped position by the application of heat and dissolving the silk and removing it from the fabric by immersing the fabric in a hot caustic solution and in a neutralizing acid bath.

6. A method of making a creped fabric wholly of nylon which comprises forming a fabric with a yarn comprising nylon combined with silk, immersing the fabric in boiling water to shrink the silk which in turn gives a creped position to the nylon, heat setting the nylon in this creped position, and dissolving the silk and removing it from the fabric by immersing the fabric in a hot caustic solution and in a neutralizing acid bath.

7. A method of making a creped fabric wholly of a nylon yarn which comprises forming a fabric comprising such nylon yarn combined with silk, boiling off the fabric and shrinking the silk which in turn gives a creped position to the nylon yarn, heat setting the nylon yarn in this creped position and dissolving the silk and removing it from the fabric by immersing the fabric in a hot caustic solution and in a neutralizing acid bath.

8. A method of making yarn wholly of nylon which comprises combining the yarn with silk, shrinking the silk to give a creped position to the nylon, heat setting the nylon in this creped position, and dissolving the silk to remove it from the yarn.

9. A method of making creped yarn wholly of nylon which comprises combining nylon yarn with silk to form a composite yarn, boiling off the composite yarn and shrinking the silk thus giving a creped position to the nylon yarn, setting the nylon yarn in this creped position by the application of heat and moisture and dissolving the silk and removing it from the nylon yarn by immersing the composite yarn in a hot caustic solution and in a neutralizing bath.

10. A method of making a creped fabric com-

prising nylon yarn which includes the steps of boiling off a fabric formed of a combined yarn of nylon and silk thereby shrinking the silk to crepe the nylon, subjecting said fabric to wet steam at a temperature in excess of the boiling off temperature, and then treating the fabric with an aqueous caustic solution to remove the silk.

11. A method of making a nylon fabric having a pebbly surface comprising the steps of boiling off a fabric made of a combined yarn of nylon and silk to shrink the silk and pebble the nylon, subjecting said fabric to wet steam at a temperature in excess of 212° F., and then treating the fabric in a caustic solution to remove the silk.

12. A method of making a creped nylon fabric comprising the steps of forming a composite yarn by throwing nylon and silk, forming said yarn into a fabric, immersing said fabric in boiling water to shrink the silk and crepe the nylon, then applying moisture at a temperature in excess of 212° F. to said fabric, and treating said fabric with caustic solution to remove the silk.

13. A method of making a crinkled nylon yarn including the steps of combining silk and nylon into a composite yarn of high twist, boiling off said composite yarn to shrink the silk and crinkle the nylon, heat setting the nylon and treating the composite yarn in a caustic solution to remove the silk.

14. A method of making a creped nylon fabric including the steps of forming a fabric of a composite yarn of nylon and silk, boiling off the fabric to shrink the silk and crepe the nylon, immersing the fabric in a boiling caustic solution to remove the silk, and treating the fabric with a neutralizing bath.

ABRAHAM L. DORGIN.

#### REFERENCES CITED

The following references are of record in the file of this patent:

#### UNITED STATES PATENTS

| Number    | Name         | Date          |
|-----------|--------------|---------------|
| 2,006,542 | Dreyfus      | July 2, 1935  |
| 2,020,907 | Rubin        | Nov. 12, 1935 |
| 2,197,896 | Miles, Jr.   | Apr. 23, 1940 |
| 2,287,099 | Hardy et al. | June 23, 1942 |
| 2,290,253 | Schneider    | July 21, 1942 |
| 2,332,738 | Meade        | Oct. 26, 1943 |

#### FOREIGN PATENTS

| Number  | Country       | Date          |
|---------|---------------|---------------|
| 552,138 | Great Britain | Mar. 24, 1943 |
| 576,050 | Great Britain | Mar. 15, 1946 |